

June 11, 1940.

E. S. DAVENPORT ET AL

2,204,209

METHOD OF HEAT TREATING STEEL AND THE METALLURGICAL PRODUCT PRODUCED THEREBY

Filed Oct. 5, 1938



INVENTORS  
EDMUND S. DAVENPORT.  
EDWIN H. ENGEL.  
BY

*John E. Jackson*  
ATTORNEY

Patented June 11, 1940

2,204,209

# UNITED STATES PATENT OFFICE

2,204,209

## METHOD OF HEAT TREATING STEEL AND THE METALLURGICAL PRODUCT PRODUCED THEREBY

Edmund S. Davenport, Chatham, N. J., and Edwin H. Engel, Vandergrift, Pa., assignors to United States Steel Corporation, a corporation of New Jersey

Application October 5, 1938, Serial No. 233,464

12 Claims. (Cl. 148—21.5)

This invention relates to metallurgy and more particularly to a method of treating steel whereby a steel article having a soft machinable exterior and relatively harder interior is obtained.

5 Heretofore in the art many methods of treating steel to obtain a hardened exterior and softer interior or core have been proposed. The present invention has an opposite objective. We have discovered that the softening rate of martensite, the ferritic form of iron characteristic of fully quench hardened steel, is much faster than that of pearlite, the ferritic form of iron characteristic of annealed or unhardened steel, and that by an appropriate heat treatment sub- 10 sequent to quench hardening we may obtain a reversal of the usual structure in a shallow hardened steel, thereby obtaining a steel product having a hardened core and softened exterior which is particularly adapted for use in the arts where 15 it is desired subsequent to hardening to subject the article to final machining, polishing, threading, shaping or the like operations before being placed into service.

20 Before further disclosing the present invention, reference should be made to the accompanying drawing wherein:

Fig. 1 illustrates in curves M, FP and P the rate of softening of martensite, fine pearlite and coarse pearlite, respectively, in terms of Brinell 25 hardness number, when heat treated at the same tempering temperature, namely, 1200° F.

Fig. 2 illustrates in curves 1, 2, 3 and 4 the hardness distribution across the diameter of a round bar in terms of Rockwell "C" hardness 30 number (1) in its quench hardened condition; (2) after heat treatment for twenty seconds at 1200° F.; (3) after heat treatment for fifty seconds at 1200° F.; and (4) after heat treatment for one hundred seconds at 1200° F.

40 Referring to Fig. 1 it may be noted that martensite (curve M) upon heat treatment at 1200° F. softens more rapidly than does fine pearlite (curve FP) or coarse pearlite (curve P) and eventually becomes the softest of the three structures. On the other hand, the coarse pearlite (curve P) which was originally the softest of the three structures eventually becomes the hardest of the three. The originally fine pearlite 45 structure ends up with an intermediate hardness.

50 Thus it will be apparent from the curves Fig. 1 that it is possible by heat treatment to alter the martensite formed by usual quench hardening methods into a relatively soft product and where there is formed by such quench hardening methods a core of either fine or coarse pearlite, the core by appropriate heat treatment may be rendered relatively harder than the originally hard martensitic surface. In ordinary quench 55 hardening methods the martensite is formed in-

wardly from the exterior surface a distance ordinarily controlled by the mass and composition of the steel and the rate of cooling applied thereto.

As an illustration of the present invention, reference should be made to the curves in Fig. 2. The steel composition of the  $1\frac{1}{16}$  inch diameter round bar treated is what is known in the art as a .74% C. steel. Such a steel may contain, for example manganese 0.30 to 0.45%, silicon 0.10 to 10 0.20% with sulphur and phosphorus in substantially residual amounts. This steel bar after being heated to a temperature at which it is fully austenitic and quenched in water (at a temperature approximating atmospheric temperature) will harden substantially as indicated in curve 1 (Fig. 2). Curve 1 shows the hardness distribution across the diameter of the steel bar. From the curve it may be noted that the center (C) of the round bar is considerably softer than 15 the outer areas (A and B).

Upon heat treatment at 1200° F. for twenty seconds (curve 2) the hardness across the diameter changed to an approximately equal value at all points which is lower than that originally 20 obtained at (C) curve 1.

Upon further heat treatment at the same temperature for a total of fifty seconds (curve 3) the exterior portion softened more rapidly than the interior and further heat treatment (curve 30 4) for a total of one hundred seconds converted the originally harder exterior (A'-B') to a much softer ferritic structure than that of the interior (C'). The hardness (Rockwell C 35) of the exterior is such as to permit ready machining, threading or polishing of the exterior area without detrimentally affecting the harder 35 interior.

The present invention offers particular advantages in the manufacture of steel shafting, 40 bolts, jail bars, machine parts and the like, wherein subsequent to hardening, final machining, cutting or threading of the surface or ends is desired before the article is ready for service use. Heretofore it has been difficult, for 45 example, in the threading of shaft or bolt ends to accomplish the threading operation subsequent to hardening, and if the threading was done prior to hardening and tempering, the threaded ends frequently warped. Moreover, in 50 prior art practice the hardness of such articles across the diameter after the tempering of the same usually approximated that indicated in curve 2 (Fig. 2) or was a compromise between 55 that of curves 1 and 2.

The practice of the present invention is applicable with appropriate modifications as to time and temperature of heat treating which is readily discernible to those skilled in the art, to a wide variety of steels and steel compositions

- known in the art as "hardening" steels wherein hardening is obtained by the formation of martensite through appropriate cooling from a temperature above the so-called "critical range." 5
- 5 In general, such steels contain carbon above about 0.25% and below about 1.50%, and may contain varying amounts of alloy constituents such as manganese, silicon, nickel, chromium, tungsten, molybdenum, titanium, zirconium, 10 copper and the like metals. These alloy constituents are permissible in the iron-carbon alloy in varying amounts before the practice of the present invention is interfered with, as one skilled in the art will recognize; for example, 15 manganese and nickel, singly or combined, are permissible in such amounts in the iron-carbon alloy as will not essentially prevent the occurrence of the transformation of austenite into ferritic structures on cooling the steel through 20 the critical range. The rate of cooling of such steels must be adjusted with respect to the percentage of these alloying constituents present to yield the hardened martensitic exterior and 25 pearlitic interior desired for heat treatment in accordance with the present invention and the precise temperature of heat treatment of the hardened product must be selected with any given steel composition to yield within an economically practical time interval the desired 30 conversion indicated in curves 3 and 4 (Fig. 2). One skilled in the art can readily ascertain these variable factors with any given transforming steel composition.

The presence of these alloying constituents frequently is desirable to impart added strength, shock resistance and the like properties to the hardened core or to impart corrosion resistance to the surface of the metal.

Having broadly and specifically identified the 40 nature and scope of the present invention and having given one specific embodiment of the same, it is apparent that many modifications and adaptations may be made of the present invention without departing essentially from the nature and scope thereof as may be included within the scope of the accompanying claims.

What we claim is:

1. The method of treating a quench hardened steel having a hardened exterior portion consisting mainly of martensite and a softer interior core consisting mainly of pearlite to render the exterior portion softer than the interior core, which comprises heating the steel to a temperature at which the rate of softening of the exterior portion is greater than the rate of softening of the interior core and maintaining the temperature until the exterior portion has acquired a hardness lower than the said core. 55

2. The method of treating a quench hardened 60 steel having a marginal martensitic area and a central pearlitic core, which comprises heating the steel to a temperature at which the rate of softening of the martensite is faster than the rate of softening of the pearlite and maintaining this temperature until the martensitic area acquires a hardness less than that of the pearlitic core.

3. The method of treating a steel having martensitic and pearlitic zones or areas to substantially reverse the hardness relationship of said zones or areas, which comprises heating said steel to a temperature at which the rate of softening of martensite is faster than the rate of softening of pearlite and maintaining said

temperature for a time interval adapted to produce a tempered martensitic structure which is softer than the simultaneously tempered pearlitic structure.

4. In the tempering of quench hardened steel, 5 the step of heating said steel to a temperature at which the rate of conversion of martensite into tempered martensite is greater than the rate of conversion of pearlite into tempered pearlite and holding the steel at said temperature for 10 a time interval effective to produce a tempered martensite softer than the tempered pearlite.

5. The method of treating a quench hardened carbon-iron alloy having an exterior area composed of martensite and an inner core area composed of pearlite, which comprises heating the same to a temperature at which the rate of softening of the martensite is greater than the rate of softening of the pearlite and maintaining the steel at this temperature until the hardness 20 of the martensitic area is less than that of the pearlitic core.

6. The method of treating a quench hardened steel containing carbon about .74% and having a marginal zone or area composed of martensite 25 and an inner core composed of pearlite, which comprises heating said steel to a temperature approximating 1200° F. for a time interval in excess of about twenty seconds until the hardness of the said marginal zone is less than the hardness 30 of said core.

7. An article of manufacture consisting of a quench hardened and tempered steel article having a pearlitic core substantially harder than the surrounding tempered martensitic structure.

8. An article of manufacture consisting of a steel article quench hardened and tempered, said article having an outer portion consisting of tempered martensite of substantially lower hardness than the inner core. 40

9. An article of manufacture, a steel article provided with an inner core area consisting of pearlite and an outer area surrounding said core consisting of tempered martensite having a hardness materially less than that of the said core. 45

10. An article of manufacture comprised of a transforming steel having a carbon content adapted to permit hardening of the same on being cooled from a temperature above the critical range to a temperature below said range, said article having an inner core area consisting substantially of pearlite and an outer area surrounding the said core area consisting of tempered martensite having a hardness materially less than that of the said core. 50

11. An article of manufacture comprised of steel, said article having a centrally located core consisting substantially of pearlite and an outer enclosing area consisting of tempered martensite having a hardness materially less than that of the core. 55

12. An article of manufacture comprised of a steel having a carbon content and an associated alloy content adapting the steel to undergo transformation and hardening on being cooled 65 through the critical range and a mass limiting the hardening to the outer portion of the article, said article being characterized by a central core consisting of pearlite and an outer portion consisting of tempered martensite having a hardness 70 materially less than that of the said core.

EDMUND S. DAVENPORT.  
EDWIN H. ENGEL.